

## 1

2,824,066

## SODIUM SOAP THICKENED SOLVENT EXTRACTED HIGH VISCOSITY INDEX OIL

John M. Musselman, Brecksville, and Cyril P. Nunley, Cleveland Heights, Ohio, assignors to The Standard Oil Company, Cleveland, Ohio, a corporation of Ohio

No Drawing. Application September 28, 1953  
Serial No. 382,845

5 Claims. (Cl. 252—42.1)

The present invention relates to a multi-purpose soda-base lubricating grease.

The grease lubricant art is one of the oldest arts known to mankind, dating back to about 1400 B. C. when greases were first used for lubricating chariot wheels. Probably, the first grease-like lubricants were animal tallow; but, when these proved unsatisfactory, further improvements were made necessary. A tremendous advance in the grease making art was made with the discovery of petroleum oil which resulted in the mineral oil greases similar to those known and used at the present time.

Ever since the inception of the first lubricating grease, grease making has been, to a large extent, an art in which the methods of cut and try have predominated. For this reason, the progress made in the manufacture of lubricating greases has been appallingly slow as compared with the development of other petroleum products. In fact, the grease making industry is still, in this present day, hampered by the lack of broad scientific knowledge which has resulted from the secrecy and mystery surrounding the activities of the skilled grease maker.

Today, practically all lubricating greases are prepared from mineral oil and a thickening or gelling agent. The oldest known thickening agents are the metallic soaps of fatty acids, such as the sodium and calcium soaps of relatively long chain fatty acids. Recently, however, other metallic soaps of fatty acids such as lithium, barium and aluminum soaps have achieved prominence as thickening agents for mineral oils. Also, in more recent years, various inorganic gelling or thickening agents have been proposed and used to some extent to replace the fatty acid soaps. Thus, we have today greases prepared from thickening agents such as silica aerogel, alumina, and various types of clays such as Attapulgus clay and bentonite.

Almost every thickening agent which has been used in the formation of a grease results in a grease which in one respect or another has superior properties. For example, the so-called soda-base greases, which are prepared from a sodium soap of a fatty acid, are known to have relatively good stability at reasonably elevated temperatures but such greases suffer the disadvantage of deteriorating rapidly in the presence of water, presumably due to the high solubility of the sodium soap in water. On the other hand, calcium soap greases are known to possess, in general, satisfactory resistance to water for most purposes, but greases prepared from calcium soaps usually have such a low melting point that they are unsuitable for use in lubricating at higher temperatures. Lithium soap greases to a large extent bridge these properties and are looked upon with some favor in the art but, since lithium soaps are relatively expensive in comparison to

## 2

sodium and calcium soaps, grease manufacturers would ordinarily prefer to employ one of the less expensive soaps. Similarly, excellent greases can be prepared from the inorganic gelling agents, hereinabove described, but again the high cost of such gelling agents is a prohibitive factor which limits the popularity of these greases.

From the preceding discussion, it is evident that the development of an inexpensive grease which does not possess the disadvantages normally attributable to calcium and sodium soap greases would be a decided boon to the art. The present invention fulfills the need for such a grease by providing a sodium soap grease which had excellent properties in the more important respects and which can be classed as a true multi-purpose grease.

In order for a grease to be classified as a multi-purpose grease, it must possess several different physical properties, the attainment of all of which simultaneously in one grease represents an exceedingly difficult achievement. One of the most important characteristics of a lubricating grease is the ability to withstand mechanical shear without undue loss in consistency, and this property is referred to as mechanical stability. Consistency is measured in terms of the penetration of the grease at 77° F. using an ASTM conical type penetrometer. In measuring the ability to withstand working, the grease is mechanically worked in an ATSM greaseworker, which consists essentially of a piston and cylinder assembly where in the piston is a flat disc having a multiplicity of relatively small perforations. The cylinder is charged with the grease to be tested, and the piston reciprocated, thus rapidly forcing the grease back and forth through the perforations of the disc. In order to measure the mechanical stability of the grease, the penetration is conventionally measured after working 0, 60, and 10,000 strokes. Ideally, the perfect grease would possess the same penetration at the beginning of the test as it possessed after being worked for 10,000 strokes but, for practical purposes, a grease is considered to have excellent mechanical stability if the gain in penetration is less than about 30.

40 The grease of our invention has this desirable property.

Another measurement of the mechanical stability of a grease is furnished by the Shell roll test which is considerably more severe than the ASTM test. In this test, the grease is packed inside a rotatable drum approximately four inches in diameter and ten inches long which contains a bar inside. Upon rotation of the drum, the grease is worked by movement of the bar and the penetration of the grease is measured before the test and at the end of the test by the Shell Microcone penetration test, Institute Spokesman (NLGI), vol. VI, No. 12, p. 1 (1943). The test is so severe that many greases will liquefy during the test so that any grease which still retains its consistency at the conclusion of the test is considered to have excellent mechanical stability. The 55 grease of our invention has excellent mechanical stability as will be seen from data hereinafter.

Another important property of a lubricating grease is its resistance to oxidation, and this is commonly referred to as oxidation stability. It has long been recognized that greases undergo certain chemical changes in storage and use. Oxidation takes place with the resultant formation of dark red or black polymers, malodor, changes in consistency, and, in certain cases, excessive oil separation. As a result, a large number of bearing manufacturers have incorporated in their specifications the requirement that the grease pass the Norma-Hoffman oxidation test. In this test, a 20 gram sample of the

grease is divided into five equal parts, each part is placed in a Pyrex dish, and the dishes are placed on racks in a vertical, cylindrical stainless steel bomb which is very similar to the induction bomb used in gasoline testing. The bomb is then immersed in a 210° F. constant temperature oil bath during the test, and the material being tested is subjected to an initial oxygen pressure of 110 p. s. i. g. (pounds per square inch gauge). The loss in pressure with time is then measured, and a loss of 5 pounds pressure in less than 100 hours is regarded as equivalent to a satisfactory stability for at least two years.

Notwithstanding the fact that our grease, unless modified, has poor oxidation stability, the grease can be given adequate resistance to oxidation by the addition of a small amount of any of the conventional antioxidants, contrary to the result that might have been expected from the use of antioxidants in greases made from acid-refined oils.

Another important property of a grease, which is often used as a criterion of the grease's ability to withstand elevated temperatures in service, is the melting point. The melting points of grease vary over a wide range. For example, the melting point of a calcium soap grease usually averages less than 200° F. while lithium and aluminum soap greases generally have melting points in the range of 350 to 400° F. The highest melting points are normally possessed by greases prepared from the inorganic gelling agents, such as bentonite, aerogels, and Attapulgus clay, and which often have melting points in excess of 400° F. Sodium soap greases, in general, normally have melting points in excess of 300° F. with the better sodium soap greases having melting points in the range of about 375 to 390° F. In summary, it can be said that any grease which possesses a melting point in excess of 400° F. has the desirable characteristic of being able to withstand relatively high temperatures during service. Our grease meets this requirement.

The water resistance of a grease is another very important characteristic since in many types of application a grease must perform its function in the presence of water whether from rain or other sources. Heretofore, calcium soap greases have been considered generally superior from the standpoint of water resistance whereas sodium soap greases have been considered notoriously poor in this respect. The first test devised by the industry for the measurement of the water resistance of a grease consisted of shaking five grams of a grease in water, and then allowing the mixture to stand while noting the time required for the grease to deteriorate. For the purposes of the present invention, this test is designated as the water immersion test. To be satisfactory in this test, a grease of grade No. 1 should have a deterioration time of at least one year. This test is met by the grease of the invention.

Another test which determines the water resistance of a grease is called the ASTM water washout test. In this test, a ball bearing is packed with the grease and a stream of water at 100° F. is played on the race of the bearing from 0.25 inch above the angular opening for one hour. The results are reported in the percent of grease retained in the bearing. In this test a rating of 60% or better is excellent. Notwithstanding the fact that our grease is a soda-base grease, which class of grease in the past has had a poor reputation on this score, our grease has satisfactory water resistance.

There is still another very important property of a grease, which heretofore has not received the full consideration that it merits, and which is termed the "dispensability" of the grease. This is the property which enables a grease to be dispensed easily from the cans, drums or other containers in which it is normally sold. It is especially important because of the fact that a

grease is normally removed from such a container by means of a pump-like attachment which withdraws the grease by vacuum.

There are two sub-characteristics which determine the dispensability of a grease. The first of these is "pumpability" which is self-explanatory. The second sub-characteristic is known as "slumpability" and of the two sub-characteristics the latter is much more difficult to achieve. The slumpability of a grease refers to the ability of a grease to level out in a container instead of adhering to the sides of a container when part of the grease is removed from the central zone of the container. The importance of this characteristic known as slumpability is apparent when one realizes that the intake tube of a pump attached to a grease container usually terminates in the center of the container near the bottom. If the grease in the container does not possess slumpability, the pump will cease to operate long before the container is empty because the grease fails to flow downward toward the intake end of the tube. The importance of dispensability is readily apparent if one visualizes the frustration of a farmer trying to pump grease out of a drum on a cold winter morning in order to get his tractor greased and started.

The measurement of slumpability is performed in an apparatus known as an E-Z Grezerator which is a piston and cylinder arrangement adapted to fit into a conventional grease container. Slumpability is measured by the amount of grease sucked into the cylinder under 21 inches of vacuum at 10° F., in a period of 15 seconds. If the grease does not possess slumpability, the intake of the cylinder will not be continually immersed in the grease and the amount of the grease sucked into the tube will be small. In this test, a rating of 120 is a perfect score and a rating of zero is the poorest score obtainable. Our grease is excellent in this important requirement.

Another important characteristic of a grease is its texture. This property is especially important because it affects the appearance of the grease and, consequently, its salability and also affects the ease of application of the grease. The desirability of a grease having a smooth and butter-like texture as contrasted to a fibrous, stringy texture for many purposes is well known. Lime greases usually have this buttery texture and the soda greases of our invention possess it in contrast to their usual fibrous texture.

It is also desirable in many cases that a grease have the property of not affecting articles of rubber with which it comes in contact. For example, rubber seals are often employed as retaining elements for grease and a grease which will act upon rubber and result in its deterioration is obviously unacceptable. It is an advantage of the grease of this invention that it does not affect such rubber seals.

It is a primary object of the present invention to provide a multi-purpose grease which, in comparison with other greases grade for grade, is excellent in all of the properties hereinabove discussed and which, in addition, is inexpensive because it utilizes a relatively cheap sodium soap as a thickening agent.

Throughout the long history of grease-making, much experimentation, involving a wide variety of oils and of soaps, has been performed in the manufacture of sodium soap greases. In this experimentation, it has continually been found that both the oil component and the soap component contribute to the final properties of the grease and that the selection of both of these components must be made with care.

Most of the experimentation with sodium soap greases had involved the use of an acid-refined oil, largely because acid refining has been an inexpensive and the most widely used method of refining. Numerous fatty acid soaps have been suggested as thickening agents for the

acid-refined oils including soaps of practically every acid from  $C_{12}$  up to  $C_{22}$  and higher, both saturated and unsaturated. However, it has never been possible to prepare from an acid-refined oil, a soda-base grease having a water resistance which even approaches the water resistance of calcium and lithium soap greases. On the other hand, it has been possible to prepare greases which have acceptable mechanical stability by employing as thickening agents sodium soaps of fatty acids which have a relatively high amount of unsaturation.

Heretofore, solvent-extracted oils have been used as components of sodium soap lubricating greases only for certain specialty purposes. Therefore, very little is known concerning the properties of greases prepared from solvent-extracted oils and it has generally been thought that the solvent-extracted oils were the approximate equivalent of the acid-refined oils in grease-making. One of the reasons why the art has generally avoided the use of solvent-extracted oils in grease-making is that the solvent-extracted oils require larger amounts of soap to thicken them and the incorporation of larger than usual amounts of soap in the oil is difficult.

The previous manufacturing experiences with acid-refined oils have furnished no guide or rule of predictability which can be followed in the manufacture of greases from solvent-extracted oils. Invariably, greases prepared from acid-refined oils and a sodium soap of a fatty acid have notoriously poor resistance to water no matter what type of acid is used in the formulation. In fact, such greases deteriorate so rapidly in water that the only known methods for evaluating water resistance can give no measurable results. From knowledge such as this, it will ordinarily be predicted that greases prepared from solvent-extracted oils and sodium soaps of fatty acids would also be notoriously poor in water resistance. We have found that this is not so when a grease is prepared from a solvent-extracted oil and the components are carefully selected.

As another instance of unpredictability it is known that, while soda-base greases prepared from acid-refined oils can be made with fairly good mechanical stability, optimum mechanical stability can be obtained only by the use, as a thickening agent, of a sodium soap of a relatively unsaturated acid and that, as a general rule, the greater the degree of unsaturation, the greater is the mechanical stability of the resultant grease. Proof of this statement has been furnished by preparing several greases from acid-refined oils each thickened with 20% by weight of a sodium soap of a fatty acid having a chain length of  $C_{18}$  with varying degrees of unsaturation from grease to grease. The procedure later to be described in Example 1 was employed and the mechanical stability of the greases was determined by the ASTM method. The data are presented in the following table:

TABLE I

| Iodine Value of Fatty Acid | Penetration Gain (10,000 strokes) |
|----------------------------|-----------------------------------|
| 0                          | 110                               |
| 20                         | 108                               |
| 40                         | 105                               |
| 60                         | 80                                |
| 80                         | 30                                |
| 100                        | 25                                |

From the data in the table, it is thus indicated that the higher the iodine value of the fatty acid, the greater the mechanical stability of the grease.

Contrasted to greases prepared from acid-refined oils, it has been found that greases which have excellent water resistance and are also excellent in the other properties hereinabove described can be prepared by combining a solvent-extracted oil of certain characteristics with a sodium soap of a fatty acid having certain, critically-defined characteristics.

In order to formulate the grease of the present invention, it has been necessary in order to obtain certain properties to proceed in directions contrary to those which might have been expected from previous knowledge on greases prepared from acid-refined oils. It is very notable, for example, and quite surprising to find that in order to obtain satisfactory and optimum mechanical stability the fatty acid from which the grease of the invention is prepared should be substantially saturated. The effect obtained by varying the degree of unsaturation of the fatty acid used in the preparation of the grease of the invention has been shown by formulating a series of greases according to the procedure of Example 1 but using  $C_{18}$  acids of varying degrees of unsaturation, and then determining the mechanical stability of the greases by the ASTM test. The data are as follows:

TABLE II

| Iodine Value of Fatty Acid | Penetration Gain (10,000 strokes) |
|----------------------------|-----------------------------------|
| 0                          | 10                                |
| 20                         | 27                                |
| 40                         | 50                                |
| 60                         | 65                                |

This data, when compared with the data in Table I, illustrates one of the differences between acid-refined oils and solvent-extracted oils in grease formulations.

In accordance with the present invention, it has been found that the grease of the invention which has all of the valuable properties hereinabove contributed to it must be prepared from the sodium soap of a fatty acid, i. e., an aliphatic hydrocarbon acid, which has the following characteristics: The acid must have an iodine value of less than 5, preferably less than 3; it must be composed of at least 80% by weight of  $C_{18}$  or higher acids, preferably at least 85% by weight; it must contain less than 20% by weight, preferably less than 15% by weight of  $C_{16}$  acids; and it must also contain less than 2% by weight, preferably less than 1% by weight of  $C_{14}$  and lower acids. There is no critical limit on the maximum chain length of the fatty acid and good results can be obtained with acids as high as  $C_{22}$ ,  $C_{24}$  or even higher. The latter figure represents a practical upper limit on the chain length.

While the above specifications may appear to encompass a large number of acids, actually only a very few acids are included since most of the acids sold commercially are mixtures of acids which do not meet the specifications. For example, the commonly used fish oil acids are too high in  $C_{14}$  and  $C_{16}$  content and too high in unsaturation. Menhaden oil, for instance, contains about 32% of  $C_{18}$  acids and 5% of  $C_{14}$  acids. Herring oil contains about 7%  $C_{14}$  acids and 27% of  $C_{16}$  acids and sardine oil contains about 4.5% of  $C_{14}$  acids and 23% of  $C_{16}$  acids. Even when hydrogenated, the fish oil acids still contain percentages of  $C_{14}$  and  $C_{16}$  acids too great to be acceptable. All available grades of commercial stearic acid, which by its name would appear to meet the characteristics, contains not more than 50% of  $C_{18}$  or higher saturated acids. In fact, there is no naturally occurring oil or fat whose fatty acid content meets the above specifications. In order to meet the specifications, it is necessary to subject a naturally occurring fat or oil through several steps of processing. For example, a fatty acid which meets the specifications can be prepared by hydrogenating fish oil acids to reduce the iodine value to the designated level and then fractionating out the lower acids so that the  $C_{14}$  and  $C_{16}$  content is reduced to an extent sufficient to meet our specifications.

The solvent-extracted oil which is combined with the sodium soap of the fatty acid of the type hereinabove defined to provide the lubricating grease of the invention need not be selected with the particularity required

for the fatty acid. However, the oil must meet certain specifications in order to be acceptable. It must have a viscosity index of at least 85, preferably at least 95; an aniline point of at least 100° C., preferably at least 115° C.; a viscosity within the range of 100 to 2,000 SSU at 100° F.; and a pour point of 10° F. or below. If desired, a pour point depressant may be used to attain the desired low pour point. The use of viscosity index improvers to meet the viscosity index specification is permissible but generally not practicable. This is because oils of low viscosity index generally also possess a low aniline point and, while a V. I. improver is capable of improving viscosity index, it will not raise the aniline point to meet our specification. In order for the oil component to be satisfactory, both the aniline point and viscosity index specifications must be met.

The preparation of the grease preferably involves the in situ formation of the fatty acid soap in the oil. A typical preparation comprises weighing the solvent-extracted oil and a calculated amount of sodium hydroxide into a mixing vessel and then heating these materials to an elevated temperature, generally in excess of 150° F., and a calculated amount of fatty acid is then weighed into the mixer. The mixer is again started and heating is continued at a temperature of approximately 300° F. After heating at the elevated temperature for about 10 to 15 minutes, until saponification is complete, an additional quantity of solvent-extracted oil is added to the mixer and heating is continued until a total processing time of about 2½ to 3 hours has elapsed. Heating is then discontinued and during the cooling of the crude grease mixture, an additional calculated quantity of solvent-extracted oil is added with the final oil addition being made at a temperature in the neighborhood of 225 to 230° F. Cooling is then continued until the grease is at a temperature suitable for packaging.

As mentioned above, the grease of the present invention requires a greater proportion of fatty acid soap than a similar grease prepared with an acid-refined oil. However, the amount of fatty acid soap is not critical and the amount of soap may be varied to provide greases of different grades, all of which, however, possess the excellent characteristics attributable to the present invention when compared with other greases of the same grade.

It is explained at this point that greases are conventionally made in several different grades according to hardness. The various grades are designated by number and range from grade No. 000 for a very soft grease up to grade No. 6 for a very hard grease. Usually, the principal difference in formulation between different grades of the same grease is that the softer greases contain less thickening agent than the harder greases. This means that generally the softer grades of grease will have different consistency than the harder grades of grease and, therefore, when one wishes to compare two or more greases of different formulation, each grease should be of the same grade. In the preparation of the grease of this invention, it has been found that a grade No. 000 grease requires about 3 to 5% of soap; a grade No. 0 grease requires about 11 to 14% by weight of soap; a grade No. 1 grease requires about 16 to 17% by weight of soap; a grade No. 2 grease requires about 24 to 25% by weight of soap; and a grade No. 6 grease requires upwards of 35% soap. From this information it can be said that the grease of the present invention preferably contains from about 3 to about 40% by weight of the fatty acid soap. The different grades of grease made by varying the soap content of the oil all possess the excellent properties attributable to the grease of the invention since variations in soap content affect only the consistency of the grease.

Other ingredients can be present in the grease by virtue of their incorporation during the preparation of the grease. It is especially desirable to incorporate a conventional amount, i. e., about 0.5 to 2% by weight of any con-

ventional oil antioxidant such as Calco MB (tetramethyl diamino diphenyl methane), Ortholeum 300, or dimethyl-para-cresol. This is so because the grease of the present invention is unusually susceptible to the affect of an antioxidant and the addition of an antioxidant results in a vast improvement in oxidation stability.

The foregoing statements concerning the addition of an antioxidant to the grease are not meant to imply that the addition of an antioxidant is in all cases essential. There are many cases in which oxidation stability is an unimportant property and in these cases the inclusion of an antioxidant may be omitted without detracting from the other properties of the grease.

The fact that the grease of the present invention is unusually susceptible to the affect of an antioxidant is another result which would not have been predictable from previous experiences using acid-refined oils in grease manufacture. It is quite well known, for example, that the improvement resulting from the addition of an antioxidant to a grease prepared from an acid-refined oil is not enough to justify the use of an antioxidant. On the other hand, the grease of the present invention when prepared without an antioxidant has relatively poor oxidation stability, but the addition of an antioxidant increases the oxidation stability to a remarkable extent so that the grease of the invention can be prepared, if desired, with an oxidation stability comparable to the majority of better greases on the market.

The invention will now be illustrated by specific examples in which parts and percentages are by weight unless otherwise specified.

#### Example 1

An oil blend was prepared by mixing together equal parts of a solvent-extracted bright stock oil having a viscosity of 150 SSU at 210° F. and a solvent-extracted neutral oil having a viscosity of 250 SSU at 100° F. There was additionally incorporated in the blend 0.5% of Paraflo, a pour point depressant, and the final oil blend was found to possess the following characteristics:

|                      |            |
|----------------------|------------|
| Pour point           | 10° F.     |
| Viscosity at 100° F. | 841.7 SSU. |
| Viscosity at 210° F. | 81 SSU.    |
| Viscosity index      | 96.3.      |
| Aniline point        | 260° F.    |

Six pounds of the oil blend and 2.8 pounds of 48-50° Baumé sodium hydroxide were weighed into a mixer. These materials were heated with agitation at 180° F. and the mixer was then stopped. There was then added 9 pounds of fatty acid (Hydrofol 150 acids) having the following characteristics:

|                    |              |
|--------------------|--------------|
| Iodine No.         | 3.0 maximum. |
| Titer              | 62 to 64° C. |
| Acid No.           | 195-201.     |
| Saponification No. | 196-202.     |

The acid was composed of about 90% stearic acid and 10% palmitic acid.

The mixer was again started and heating continued to about 295 to 300° F. The temperature was held at about 300° F. for 10 to 15 minutes and after a total processing of about 60 minutes, 10.5 pounds more oil and 0.35 pound Calco MB were weighed into the mixed mixer over a period of about 20 to 30 minutes causing a drop of about 20° F. in the temperature. Heating was continued until a temperature of about 295 to 300° F. was again reached, controlling the temperature rise so as to reach the desired temperature after about 160 minutes total processing time. At this point, heating was stopped and cooling started, along with the addition of 10.5 pounds of additional oil blend. When the mixture had cooled to 225 to 230° F., the final oil addition (6.5 pounds) was made, with the addition of oil being completed before the mixture was below 210° F. Agitation

and cooling were continued until the grease was at a temperature of 160° F. The mixer was then stopped and the grease withdrawn.

The grease of this example had a soap content of approximately 23%. It possessed an initial penetration at 77° F. of about 290 and after 10,000 strokes working in the ASTM greaseworker, the penetration rose to only 300, a gain of about 10. The melting point of the grease was in excess of 400° F. and in the Norma-Hoffman oxidation test, there was a pressure loss of only about one pound after 100 hours. In addition, the grease possessed excellent water resistance (a deterioration time of more than one year by the water immersion test) and good dispensability. It also possessed an excellent texture being smooth and buttery as contrasted to a fibrous, stringy texture. It also rated excellent in the E-Z Grezerator test.

A repetition of the example in which the antioxidant was omitted resulted in a grease which had a pressure loss of 100 pounds in the Norma-Hoffman oxidation test. This shows the value of an antioxidant in our grease.

#### Example 1-A

A grease was prepared according to the exact procedure of Example 1 with one exception. A saturated fatty acid having an average chain length two carbon atoms less than the acids employed in Example 1 was used. The resultant grease possessed much poorer water resistance (3 to 4 months by the water immersion test) than the grease of Example 1 and thus the grease is not classifiable as a multi-purpose grease.

#### Example 1-B

A grease was prepared according to the exact procedure of Example 1 with one exception. A fatty acid having the same average chain length as the Hydrofol 150 acids but having an iodine value of about 50 was substituted for the Hydrofol 150 acids. The resultant grease was much poorer in mechanical stability than the grease of Example 1, showing an average penetration gain of about 60 after 10,000 strokes working. The water resistance of the grease was also poor, about 20% of the grease being retained in the ASTM water washout test. This grease thus fails as an all-purpose grease.

#### Example 1-C

A grease was prepared according to the exact procedure of Example 1 with one exception. A blend of acid-refined oils which possessed approximately the same viscosity and pour point as the blend of solvent-extracted oils employed in Example 1 was substituted for the latter. The resultant grease was decidedly poorer than the grease of Example 1 particularly in regard to water resistance and mechanical stability. In the water immersion test almost immediate deterioration was noted and in the ASTM greaseworker test, a penetration gain of about 110 was noted after 10,000 strokes. These facts show that this grease fails as a true multi-purpose grease.

The results of Examples 1-A, 1-B and 1-C illustrate the sensitivity of the grease of the invention (Example 1) to changes in formulation which result in a grease outside the scope of the invention. Example 1-A shows that fatty acids of shorter chain length than that specified are not suitable because the resultant grease possesses very poor water resistance. Example 1-B shows that the use of a fatty acid of high iodine value seriously detracts from the mechanical stability and water resistance of the grease and Example 1-C demonstrates the relatively poor qualities of a grease prepared from an acid-refined oil and the soap used in the present invention.

#### Example 2

A grease was prepared according to the procedure of Example 1 with one exception. There was substituted for the Hydrofol 150 acids used in Example 1 an equal

quantity by weight of Hydrofol AB acids with suitable adjustment of the caustic. Hydrofol AB acids contain about 13.5% palmitic acid, 17.2% stearic acid, 38.3% arachidic acid, 29.2% behenic acid and 1.8% myristic acid. The maximum iodine value is 5 and the average chain length is about C<sub>20</sub>.

The resultant grease possessed even better mechanical stability and water resistance than the grease of Example 1. It was also excellent with respect to oxidation stability, texture, dispensability, and had a melting point in excess of 400° F.

#### Example 3

A grease was prepared according to the procedure of Example 1 with the following exceptions: A solvent-extracted bright stock oil having a viscosity of 750 SSU at 100° F. was substituted for the oil blend used in Example 1. The bright stock oil had an aniline point of about 246° F., a pour point of 0° F., and a viscosity index of 95. Also, the amount of fatty acid and caustic was increased so that the finished grease had a soap content of 27%. The result was a grade No. 2 grease of excellent characteristics. The penetration gain after 10,000 strokes working in the ASTM greaseworker was only 1. In the ASTM water washout test 74% of the grease was retained. The melting point was over 400° F.

#### Example 4

A grease was prepared according to the procedure of Example 1 with the following exceptions: For the oil blend used in Example 1 there was substituted a blend of three oils, including the solvent-extracted bright stock oil used in Example 3 in the amount of 51.3% of the finished grease, a solvent-extracted neutral oil having a viscosity of 140 SSU at 100° F., an aniline point of 220° F. and a pour point of 0° F. in the amount of 17.3% of the finished grease, and a solvent-extracted neutral oil having a viscosity of 330 SSU at 100° F., a pour point of 0° F., and an aniline point of 230° F. in the amount of 17.3% of the finished grease, the viscosity index of the blend exceeding 95. The amounts of fatty acid and caustic were reduced to provide a finished grease having a soap content of about 13.6%. The result was a grade No. 0 grease of excellent characteristics. It possessed a rating of 60.5% in the ASTM water washout test and in the ASTM greaseworker test it showed a penetration gain of only 4 after 5,000 strokes. The melting point of the grease exceeded 400° F. The grease possessed a slumpability rating of 113 which is excellent.

#### Example 5

A grease was prepared according to the procedure of Example 3 with one exception: The amounts of fatty acid and caustic were reduced to provide a finished grease having a soap content of about 16.4%. The result was a grade No. 1 grease of excellent characteristics.

#### Example 5-A

The grease of Example 5 was compared extensively with a number of competitive greases prepared not only from sodium fatty acid soaps but also from other metal soaps and from inorganic gelling agents. The tests upon which the comparisons were based include melting point; mechanical stability, including both the ASTM greaseworker test and the Shell roll test; water resistance by the ASTM water washout test; and slumpability as measured by the E-Z Grezerator. The results of these comparative tests are presented in the following table which also includes a description of the various greases. All greases except that of Example 4 and the last grease in the table are greases prepared and sold commercially at the present time and are representative of the best products produced by leading oil companies in this country.

TABLE III

| Grease Description     |                                                     | Thickening Agent                                   | Melting Point, °F. | ASTM Grease-worker Test, Penetration |                              | Shell Roll Test, Penetration |               | ASTM Water Washout Test, Percent Grease Retained | Slumpability, E-Z Grezerator |
|------------------------|-----------------------------------------------------|----------------------------------------------------|--------------------|--------------------------------------|------------------------------|------------------------------|---------------|--------------------------------------------------|------------------------------|
| Source                 | Oil Component                                       |                                                    |                    | Initial                              | After 10,000 Strokes         | Initial                      | After Working |                                                  |                              |
| Example 4              | Solvent-Refined oil, 770 SSU at 100° F., 94 V. I.   | Sodium soap saturated C <sub>18</sub> acids, 16.4% | 400+               | 356                                  | 354 (5,000 strokes). Gain=0  | 197                          | 235-----      | 69.3                                             | 100—Good.                    |
| Commercial Grease #1   | Acid-Refined oil, 400 SSU at 100° F., 70 V. I.      | Sodium soap, 14%.                                  | 350                | 338                                  | 357 (5,000 strokes). Gain=19 | 180                          | liquid-----   | 43.4                                             | 55—Average.                  |
| Commercial Grease #2   | 2,000 SSU at 100° F., 70 V. I.                      | Calcium soap, 5%.                                  | 190                | 308                                  | 348 Gain=40                  | 250                          | do-----       | 57.9                                             | 47—Fair.                     |
| Commercial Grease #3   | 500 SSU at 100° F., 52.1 V. I.                      | Calcium soap, 9.7%.                                | 190                | 332                                  | 360 Gain=28                  | 178                          | 193-----      | 46.34                                            | 0—Poor.                      |
| Commercial Grease #4   | 257 SSU at 100° F., 71 V. I.                        | Lithium soap, 9.1%.                                | 350-400            | 307                                  | 356 Gain=49                  | 170                          | 221-----      | 57.4                                             | Do.                          |
| Commercial Grease #5   | 535 SSU at 100° F., 35 V. I.                        | Lithium soap, 10.5%.                               | 350-400            | 256                                  | 328 Gain=72                  | 120                          | 205-----      | 54.6                                             | 5—Poor.                      |
| Commercial Grease #6   | 1,247 SSU at 100° F., 59 V. I.                      | Aluminum soap, 5.6%.                               | 190-220            | 312                                  | 356 Gain=44                  | 171                          | 291-----      | 43.24                                            | 6—Poor.                      |
| Commercial Grease #7   | 471 SSU at 100° F., 48 V. I.                        | Barium soap-----                                   | 350                | 310                                  | 364 Gain=54                  | 170                          | liquid-----   | 27.4                                             | 30—Poor.                     |
| Commercial Grease #8   | 1,374 SSU at 100° F., 11.6 V. I.                    | Bentonite-----                                     | 400+               | 328                                  | 341 Gain=13                  | 157                          | 191-----      | 66.49                                            | 56—Average.                  |
| Experimental Grease #9 | Solvent-Extracted oil, 800 SSU at 100° F., 94 V. I. | Attapulgus Clay.                                   | 400+               | 325                                  | 321 Gain=0                   | 186                          | 175-----      | 35.6                                             | 126—Excellent.               |

From a study of the table, the outstanding all-around characteristics of the grease of the invention are apparent. For example, it is to be noted that the competitive sodium soap grease is markedly deficient in water resistance; the lithium soap greases are poor in dispensability and mechanical stability; the calcium soap greases are exceptionally low melting; the aluminum grease has poor water resistance and dispensability; the barium soap grease is poor in many properties; only the greases prepared from a bentonite clay and Attapulgus clay even approach the properties of the grease of the invention.

From the foregoing description of the invention, it can be seen that by selecting a particular solvent-extracted oil and by even more particularly selecting a particular type of fatty acid from the vast number of oils and fatty acids which have been suggested as components of lubricating greases, the present invention provides an inexpensive grease of exceptionally good characteristics which renders it useful for many varied purposes. Thus, the invention is seen to reside in a combination of particular ingredients which is believed to be novel.

Many modifications within the scope of the invention may be made by those skilled in the art. For example, it is possible to incorporate in the grease any of the known additives or fillers in order to produce a superior grease for a special purpose. The term "consisting essentially of" as used in the appended claims does not exclude the presence of substances such as these which do not alter the basic and novel characteristics of our grease.

It is obvious that many such changes and modifications in various details of the invention can be made without departing from the spirit thereof. Accordingly, the invention is to be limited only by the scope of the appended claims.

We claim:

1. A multi-purpose lubricating grease consisting essentially of from about 60 to about 97% by weight of a solvent-extracted mineral oil having a viscosity of about 100 to 2000 S. S. U. at 100° F., a pour point at least as low as about 10° F., a viscosity index of at least 85, and an aniline point of at least 100° C., said oil being thickened with the sodium soap of a fatty acid in the amount of about 3 to about 40% by weight of the grease, the fatty acid being composed of at least 80% by weight of C<sub>18</sub> and higher acids, less than 20% by weight of C<sub>16</sub> acids and less than 2% by weight of C<sub>14</sub> and lower acids, the amount of unsaturated acids being sufficiently low to provide an iodine value of less than 5.

2. A multi-purpose lubricating grease consisting essentially of from about 60 to about 97% by weight of a solvent-extracted mineral oil having a viscosity of about 100 to 2000 S. S. U. at 100° F., a pour point at least as low as 10° F., a viscosity index of at least 95, and an aniline point of at least 115° C., said oil being thickened with the sodium soap of a fatty acid in the amount of about 3 to about 40% by weight of the grease, the fatty acid being composed of at least 85% by weight of C<sub>18</sub> and higher acids, less than 15% by weight of C<sub>16</sub> acids and less than 1% by weight of C<sub>14</sub> and lower acids, the amount of unsaturated acids being sufficiently low to provide an iodine value of less than 3.

3. A lubricating grease according to claim 1 which contains a minor percentage of an oil antioxidant to improve the oxidation stability of the grease.

4. A grease according to claim 1 in which the fatty acid is composed of about 90% stearic acid and about 10% palmitic acid, and in which there is incorporated an amount of tetramethyl diamino diphenyl methane to improve the oxidation stability of the grease.

5. A grease according to claim 1 in which the fatty acid is composed of about 38-39% arachidic acid, 29-30% behenic acid, 17-18% stearic acid, 13-14% palmitic acid, and traces of unsaturated acids and in which there is incorporated tetramethyl diamino diphenyl methane in an amount to improve the oxidation stability of the grease.

#### References Cited in the file of this patent

#### UNITED STATES PATENTS

|           |                  |                |
|-----------|------------------|----------------|
| 1,989,196 | Hilliker         | Jan. 29, 1935  |
| 2,229,367 | Brunstrum et al. | Jan. 21, 1941  |
| 2,318,847 | Flint et al.     | May 11, 1943   |
| 2,428,123 | Morgan et al.    | Sept. 30, 1947 |
| 2,534,053 | O'Halloran       | Dec. 12, 1950  |
| 2,588,280 | O'Halloran       | Mar. 4, 1952   |
| 2,595,556 | Worth et al.     | May 6, 1952    |
| 2,598,154 | Bailey et al.    | May 27, 1952   |
| 2,626,896 | Dilworth et al.  | Jan. 27, 1953  |
| 2,626,898 | Dilworth et al.  | Jan. 27, 1953  |

#### OTHER REFERENCES

Manufacture and Application of Lubricating Greases, Boner, Reinhold Pub. Co., N. Y. (1954), pp. 157-8.

Chemical Refining of Petroleum, Kalichevsky and Stagner, Reinhold Pub. Co., 2nd ed. (1942), p. 72.